

J. C. KING,  
ELECTRODE AND PROCESS OF MAKING SAME,  
APPLICATION FILED MAY 22, 1916.

1,312,255.

Patented Aug. 5, 1919.



FIG. 1.



FIG. 3.



FIG. 2.



FIG. 4.



FIG. 5.

Witnesses

S. R. Wallen  
G. L. Moreland

Inventor

J. C. King  
By  
Letherton Haught Co  
Attn: S

# UNITED STATES PATENT OFFICE.

JESSE CRITZ KING, OF MONTREAL, QUEBEC, CANADA.

## ELECTRODE AND PROCESS OF MAKING SAME.

1,312,255.

Specification of Letters Patent. Patented Aug. 5, 1919.

Application filed May 22, 1916. Serial No. 99,104.

To all whom it may concern:

Be it known that I, JESSE CRITZ KING, a citizen of the United States, and resident of the city of Montreal, in the Province of Quebec and Dominion of Canada, have invented certain new and useful Improvements in Electrodes and Processes of Making Same, of which the following is a full, clear, and exact description.

10 This invention relates to the manufacture of electrodes for use in electric furnaces and the like.

These electrodes are subject to considerable wasting away by burning under the action of air or other oxidizing gases between the carbon holders of the furnace electrodes and the smelting hearth. If the electrode is not protected by some means, the portion exposed to the air wastes away very rapidly.

20 Several methods have been proposed to prevent this, namely, by covering the surface of the electrode with a fireproofing material reinforced or held in position by wire fabric or other reinforcement; by electroplating a metal coating upon the surface of the electrode; by covering the electrode with an enamel or some form of paste; by converting the surface of the electrode into carbide or into graphite; or by pressing granular material, which would resist or retard oxidation, into the surface of the electrode. All of these methods have, however, failed to a large extent when the material has been subjected to the action of the air and gases

35 and to the stresses caused by expansion and contraction at the high temperatures of the electric furnace, this failure being largely due to poor bonding of the material to the smooth surface of the electrode.

40 Heretofore, electrodes have been pressed or squirted through a smooth die or formed in a mold having a smooth wall, which delivered a finished electrode having a substantially smooth surface, to which any protective substances adhered with great difficulty, especially when subjected to very high temperatures.

The main object of my invention is to provide a simple and inexpensive method of producing an electrode having a roughened surface to which a suitable coating will readily adhere.

In the drawings which illustrate my invention:—

55 Figure 1 is an elevation showing the elec-

trode with the protective covering in position on the core.

Fig. 2 is a plan view of same.

Fig. 3 is a view showing the electrode with the roughening means partly removed. 60

Figs. 4, 5, are views showing alternative forms.

In carrying out my invention in its preferred form, I employ a mold 9 lined with wire fabric 10 or other suitable material 65 adapted to form irregularities upon the surface of the electrode or core. The mold is then filled with some form of carbon in a plastic condition, and an electrode of the desired shape, size and length is produced. 70 This electrode, when set or hardened, is removed and the wire fabric or like material is stripped from its surface, leaving same roughened by numerous irregular grooves 11, which are adapted to form keys to hold 75 the coating material with which it is afterward covered. This irregular grooved surface is then covered with a layer of paste 12, formed preferably of a mixture of fire clay and graphite, or other suitable non-oxidizing 80 material, to the desired thickness. The electrode is then baked or dried to remove any water or gases, and the plastic coating is firmly bonded on to the electrode.

It will be obvious that many modifications of the above method may be employed to produce the core of an electrode having a roughened or grooved surface, to which a non-oxidizing coating may be applied. In

Fig. 4, I have shown a mold having its inner surface provided with ridges 13, which may be formed spirally or otherwise, and which are adapted to produce an electrode having a grooved surface to which the non-oxidizing coating may be applied. This 95 mold will consist of a plurality of parts suitably held together, while the core is being formed, and adapted to be separated and removed without breaking or deforming the core itself. The mixture of fire clay and graphite may then be pressed, plastered or sprayed upon the surface of the electrode into the grooves to form a coating or layer, which when baked with the electrode becomes virtually an integral part thereof, and 100 will stand very high temperatures and other stresses.

In Fig. 5, I have shown a mold provided with recesses or grooves 14, which will form projections or ridges on the surface of the 110

core of the electrode. The non-oxidizing protective material may then be applied to this roughened surface and will be bonded on to the electrode when same is finally 5 baked.

Other methods of roughening, grooving or ridging the surface of the electrode core may be employed without departing from the spirit of this invention. The non-oxidizing 10 protective covering may be applied to the roughened surface of the electrode core in any suitable manner, by pressing, spraying or plastering, or it may be molded on to the surface, using the electrode as a core within 15 a suitable mold.

Although I prefer to bake the non-oxidizing coating with the core in an oven in a single operation, the carbon core may be formed with its roughened surface and 20 baked, and the protective covering may be afterward applied and baked or dried on to the surface in a separate operation, the essential feature of the invention being the production of an electrode having a roughened, grooved or ridged surface with a protective covering applied thereto in such a manner as to produce an electrode having the core and surface covering integral and firmly bonded to resist high temperatures 25 and other stresses to which it may be subjected.

Having thus described my invention, what I claim is:—

1. An electric furnace electrode having a 35 roughened surface, and a protective coating overlying and baked on to the surface of the electrode, substantially as described.

2. As a new article of manufacture, an electric furnace electrode having a roughened surface, and a non-oxidizing coating of fire clay and graphite bonded into the roughened surface of the electrode, substantially 40 as described.

3. A method of making electric furnace 45 electrodes, which consists in lining a mold with a fabric of suitable material, filling the mold with plastic carbon, withdrawing the electrode, removing the fabric from the surface of the electrode whereby such surface 50 is left in roughened condition, and then

covering the surface of the electrode with a non-oxidizing protective material.

4. A method of making electrodes, which consists in bringing the material of the electrode while in plastic condition into and out of contact with a roughening element of woven wire whereby the surface of the material is roughened, and then coating such roughened surface with a non-oxidizing protective coating. 55

5. A method of making electrodes, which consists in bringing the material of the electrode while in plastic condition into and out of contact with a roughening element of woven wire whereby the surface of the material is roughened, then coating such roughened surface with a non-oxidizing protective coating, and then baking the electrode and coating whereby the two are inseparably bonded together. 60

6. The process of making electrodes which consists in roughening the surface of an unbaked electrode, applying a protective coating thereon overlying said roughened surface and of substantial thickness, and baking the electrode and the coating to drive off the volatile constituents. 70

7. The process of making carbon electrodes for electric furnaces which consists in roughening the surface of an unbaked electrode, applying thereon to overlie said roughened surface a plastic protective coating, and baking the electrode and the coating to drive off the volatile constituents. 80

8. The process of making carbon electrodes for electric furnaces which consists in molding an electrode having a roughened surface, applying thereon a plastic protective coating, and simultaneously baking the electrode and the coating to drive off 90 the volatile constituents contained in the electrode and the coating, and inseparably bond the two together.

In witness whereof, I have hereunto set my hand, in the presence of two witnesses. 95

JESSE CRITZ KING.

Witnesses:

C. W. TAYLOR,  
G. M. MORELAND.